

## UNITED STATES PATENT OFFICE

2,183,391

## ALUMINUM BASE ALLOY

Otto Dahl, Berlin-Wilmersdorf, and Herbert Dallmann, Berlin-Karlshorst, Germany, assignors to General Electric Company, a corporation of New York

No Drawing. Application August 30, 1938, Serial No. 227,594. In Germany September 1, 1937

3 Claims. (Cl. 75—142)

Aluminum and its alloys are, as well known, exceedingly sensitive to the action of mercury, which metal forms an amalgam with aluminum. This amalgam prevents the formation on the 5 aluminum of a dense closely adhering oxide film; in view of the base-metal characteristic of aluminum, this oxide film constitutes the only protection which that metal has against the destructive effect of air, oxygen or water. Because of 10 this, a piece of aluminum or aluminum alloy will, once it has been in contact with mercury, oxidize much more rapidly when exposed to air, or will be more quickly destroyed when exposed to water. In view of this, users are always cautioned against 15 bringing aluminum and aluminum alloys in contact with mercury, or against using aluminum and aluminum alloys where there is a possibility of contact with mercury due to operating disturbances or accident. For instance, no mercury 20 thermometers can be used in fermenting vats which are made of aluminum, or special effort must be taken in order that when the thermometer is accidentally destroyed, the mercury will not come in contact with the aluminum. Up to 25 the present it was out of the question to use aluminum or aluminum alloys in permanent contact with mercury and water, such as would be required for the floats of some measuring instruments.

30 It has been found surprisingly, that such a contact may be well permitted, and that contacts with aluminum alloys could be well applied to such a purpose, provided the alloys are suitably chosen. The required resistance to corrosion is obtained by alloying to the aluminum metals such as copper, magnesium and manganese. The mere addition of copper is of considerable influence on the resistivity against mercury. An addition of one 0.1 per cent reduces 35 the oxide formation considerably, and with additions of 0.5 per cent the alloy will be practically resistant to mercury the resistance increasing with a further increase in the copper content. In these cases, however, where the alloy comes 40 simultaneously in contact with water or salt solutions, the effect of higher copper additions cannot be utilized, since it is known that the higher copper content considerably reduces the resistance to corrosion in regard to watery solutions and moist 45 atmosphere.

50 Manganese acts along the same lines as copper. An addition of 1 per cent of manganese may be considered as equivalent to an addition of 6.5 per cent of copper. If both elements are added 55 simultaneously, their effects become apparently

additive. In those cases where a corrosion due to moisture or salt solution must be guarded against, besides corrosion due to mercury, the addition of manganese will be preferable for the reason mentioned above. The total content of manganese and copper in the alloy should not materially exceed 5 per cent.

Besides, the resistance against corrosion caused by watery corrosive agents can be further increased by an addition of magnesium, a metal 10 which increases the resistance of aluminum against these corrosive effects. However, as the experiments on which the application is based have shown, an addition of magnesium will decrease at the same time the resistance with regard to mercury, that is to say, it partly offsets the influence of the copper or manganese respectively which has been added. For this reason, the maximum magnesium addition cannot be resorted to, and one must be satisfied with magnesium 15 contents of approximately 1 to 4 per cent. In this manner, alloys are obtained which are so resistant to mercury and water, even if they are exposed to continuous simultaneous contact with these agents, that they can be used for floats and 20 similar parts. The alloy composition of 2 per cent of magnesium, 0.5 per cent of copper, 1 per cent of manganese, iron and silicon in their usual 25 limits, the remainder being aluminum, has proved to be well suited for the above purposes.

If no danger of corrosion by moist air or salt 30 solution exists, the addition of magnesium may be omitted, and in this case the manganese and especially the copper content may be higher. As in most cases where an increase in the general 35 resistance is attained by means of alloy additions, the sensitivity with respect to action at the grain boundaries will increase, even with the alloys which we have here stated. This action at the grain boundaries can become especially dangerous 40 when the parts in question are subject to internal stresses, which originate either from the casting process or from the cold working. For this reason, such parts must be annealed prior to their 45 utilization so as to remove any internal tension.

It is known that the resistance with respect to 50 mercury is raised by the addition of copper, but it was not known that absolutely permanent alloys can be obtained in this manner. It is also known that the resistance with respect to salt solutions is increased by the addition of magnesium; but it was not known that the simultaneous addition of copper and magnesium, possibly together with manganese, will create alloys which remain quite 55 stable even when exposed to simultaneous con-

tact with mercury and watery solutions. In order to give additional protection to the parts which have been alloyed according to the above data, an additional surface protection may be procured by means of oxidation, which may be accomplished with or without electric current.

What we claim as new and desire to secure by Letters Patent of the United States, is:

1. An aluminum base alloy subject to oxidizing conditions and contact with mercury, said alloy containing more than 0.3 per cent but not more than 1.5% copper, more than 0.3 per cent manganese, and 0.5 to 4 per cent magnesium, the remainder of said alloy consisting of aluminum, and the total content of copper and manganese being not greater than 5 per cent by weight of the alloy.

2. An aluminum base alloy subject to oxidizing conditions and contact with mercury, said alloy containing an appreciable quantity but not more than 1.5 per cent copper, 0.3 to 1 per cent manganese, 0.5 to 4 per cent magnesium with the remainder aluminum. 5

3. An aluminum base alloy subject to oxidizing conditions and contact with mercury, said alloy containing 0.3 per cent but not more than 1.5 per cent copper, at least 0.3 per cent manganese, 10 the total content of copper and manganese being not greater than 5 per cent by weight of said alloy, the remainder of said alloy consisting of aluminum.

OTTO DAHL.  
HERBERT DALLMANN.

15

CERTIFICATE OF CORRECTION.

Patent No. 2,183,391.

December 12, 1939.

OTTO DAHL, ET AL.

It is hereby certified that error appears in the printed specification of the above numbered patent requiring correction as follows: Page 1, first column, line 3, for "almalgam" read amalgam; line 26, for "alluminum" read aluminum; line 39, for the word "one" read only; same page, second column, line 38, for "boudaries" read boundaries; line 48, for "allows" read alloys; and that the said Letters Patent should be read with this correction therein that the same may conform to the record of the case in the Patent Office.

Signed and sealed this 30th day of January, A. D. 1940.

Henry Van Arsdale,  
Acting Commissioner of Patents.

(Seal)